

# UNITED STATES PATENT OFFICE.

ROBERT A. HADFIELD, OF SHEFFIELD, ENGLAND.

## METHOD OF TREATING STEEL ARMOR-PLATES, &c.

No. 802,188.

Specification of Letters Patent.

Patented Oct. 17, 1905.

Application filed June 28, 1905. Serial No. 267,344.

To all whom it may concern:

Be it known that I, ROBERT A. HADFIELD, a subject of the King of Great Britain, and a resident of Sheffield, county of York, England, 5 have invented an Improvement in Methods of Treating Steel Armor-Plates, &c., of which the following description is a specification.

This invention has reference to an improved manufacture or treatment of steel for the purpose of increasing the toughness thereof, and is specially applicable to the treatment of nickel chromium steel, whether containing tungsten or not, such as is described in the specification of British Letters Patent granted 15 to me, No. 16,132 of 1901.

The invention may be advantageously applied to the treatment of armor-plates and other articles of steel in the form of castings.

According to one method of carrying out 20 my invention the article—for example, a cast armor-plate of steel of the kind referred to—is heated uniformly to a temperature of from about 950° C. (nine hundred and fifty degrees centigrade) to about 1,100° C. (eleven hundred degrees centigrade) and then cooled, preferably in air, which avoids sudden cooling such as would result if the article were quenched in a hardening liquid. It is then reheated to a temperature of about 700° C. 25 (seven hundred degrees centigrade) and cooled slowly, preferably in the furnace in which the heating was previously effected, after which it is again heated to a temperature of about 700° C. (seven hundred degrees centigrade) and allowed to cool slowly to a temperature of about 640° C. (six hundred and forty degrees centigrade,) whereupon it is suddenly cooled, as by quenching in water—for example, by complete immersion in water or by 30 spraying with water or by an air-blast, but preferably in water. It is then reheated to about 600° C. (six hundred degrees centigrade) and again suddenly cooled as before, preferably by quenching in water.

45 According to a modified method the first-mentioned reheating operation to about 700° C. (seven hundred degrees centigrade) followed by slow cooling is omitted, the method in other respects being like that hereinbefore described.

One or both faces of cast nickel-chromium-steel armor-plates treated as described can, if desired, be afterward cemented and subsequently hardened in the usual way.

55 It is to be understood that the invention is

not limited to the employment of the particular temperatures mentioned, as these may sometimes and with advantage be varied to a small extent. For example, the reheating in each case may be carried to from about 700° C. to 720° C. (seven hundred to seven hundred and twenty degrees centigrade.) Instead of slowly cooling to about 640° C. (six hundred and forty degrees centigrade) after reheating, the cooling may advantageously be carried down only to 655° C. (six hundred and fifty-five degrees centigrade,) and sometimes, as when dealing with large masses of steel or cemented plates, it is desirable when suddenly cooling the metal to carry such sudden cooling to a point not below, say, about 250° C. (two hundred and fifty degrees centigrade) in order to avoid any cracking of the metal. Also the final reheating may be carried to about 620° C. (six hundred and twenty degrees centigrade.)

Steel treated in either of the ways described is found to possess excellent toughness, which renders it specially suitable for the manufacture of armor-plates, shields, and other articles, including safes or parts of safes. Satisfactory results have been obtained by treating in each of the ways hereinbefore described cast nickel-cromium-steel armor-plates containing from about .3 % (decimal three per cent.) to .4 % (decimal four per cent.) of carbon, about .25 % (decimal two five per cent.) of manganese, about 1.8 % (one decimal eight per cent.) of cromium and about 3.3 % (three decimal three per cent.) of nickel, the plate being made from steel produced in the manner described in my said former specification and cast in a sand mold and having a thickness of about six inches. Such a six-inch plate attacked by common lyddite and armor-piercing projectiles of 4.7" and 6" (four decimal seven and six inch) calibers has withstood over fifteen thousand foot tons of energy without showing a single crack. Also a four-inch plate treated as described and having a carbonized or cemented face has successfully withstood the attack of a 4.7" (four decimal seven inch) caliber armor-piercing shell. Steel treated as hereinbefore described is also capable of successfully withstanding excessive 95 vibrating shocks, and is therefore adapted for the construction of parts of machines, also gun-carriage parts that are liable to be subjected to such shocks, and parts designed for 100 many other purposes.

Having fully described my invention, what I claim as new, and desire to secure by Letters Patent, is—

1. The herein-described process of toughening steel, comprising the steps of uniformly heating the steel to a temperature up to and over 950° centigrade, and then cooling; reheating the cooled steel to a temperature of from about 700° to 720° centigrade; cooling slowly to a temperature of about 640° centigrade and then quickly cooling the same; reheating the steel to about 600° centigrade, and finally quickly cooling the same.
2. The herein-described process of toughening steel, comprising the steps of uniformly heating the steel to a temperature of 950° centigrade and above, but not over 1,100° centigrade, and then cooling; reheating the cooled steel to a temperature of from 700° to 720° centigrade and cooling slowly to about 640° centigrade; then quickly cooling the steel; reheating to about 600° centigrade, and finally quickly cooling.
3. The herein-described process of toughening steel, comprising the steps of uniformly heating the steel to a temperature up to and above 950° centigrade and cooling slowly; reheating the steel to a temperature of about 700° centigrade and cooling slowly; again raising the temperature of the steel to about 700° centigrade and then cooling slowly to about 640° centigrade; then quickly cooling; reheating the cooled steel to about 600° centigrade, and finally quickly cooling the same.
4. The herein-described process of toughening steel comprising the steps of uniformly heating the steel to a temperature up to and over 950° centigrade, and then cooling; reheating the cooled steel to a temperature of from about 700° to 720° centigrade; again

raising the temperature of the steel to from 700° to 720° centigrade and cooling slowly to from 655° to 640° centigrade and then quickly cooling to about 250° centigrade; reheating to from 600° to 620° centigrade, and finally quickly cooling the steel. 45

5. The herein-described process of treating armor-plates of nickel chromium steel, comprising the steps of heating the plate uniformly up to a temperature of from about 950° to about 1,100° centigrade, and cooling slowly; reheating the cooled plate to a lower temperature, but not higher than 720° centigrade; cooling the plate slowly to a temperature of from 655° to 640° centigrade and then 55 suddenly cooling; again reheating to a temperature not higher than about 620° centigrade, and suddenly cooling the plate.

6. The herein-described process of treating armor-plates of cast nickel chromium steel 60 containing from 0.3 per cent. to 0.4 per cent. of carbon, about 0.25 per cent. of manganese, about 1.8 per cent. of chromium, and about 3.3 percent. of nickel, comprising the steps of raising the temperature of the plate to from 65 about 950° to about 1,100° centigrade, and cooling slowly, reheating the cooled plate to a lower temperature of about 700° centigrade; cooling the plate slowly to about 640° centigrade and then suddenly cooling; again reheating to a temperature of about 600° centigrade, and finally suddenly cooling the plate. 70

In testimony whereof I have signed my name to this specification in the presence of two subscribing witnesses.

ROBERT A. HADFIELD.

Witnesses:

EUSTACE H. BURKE,  
LESLIE E. WHEELER.